

Sept. 2, 1930.

R. SERGESON

1,774,999

METHOD OF HEAT TREATING NITRIDED ARTICLES

Filed Sept. 20, 1929



Fig. 2



Fig. 1



Fig. 3



Fig. 4

Inventor

Robert Sergeson

By

William Ieler  
Attorney

## UNITED STATES PATENT OFFICE

ROBERT SERGESON, OF MASSILLON, OHIO, ASSIGNOR, BY MESNE ASSIGNMENTS, TO  
REPUBLIC STEEL CORPORATION, OF YOUNGSTOWN, OHIO, A CORPORATION OF NEW  
JERSEY

## METHOD OF HEAT TREATING NITRIDED ARTICLES

Application filed September 20, 1929. Serial No. 384,102.

This invention relates in general to the nitriding of alloy steel articles and more particularly to a novel heat treatment for the nitrided articles, whereby brittleness of the nitrided case is more or less completely eliminated, and the toughness of the case increased to a considerable extent.

According to Fry, a well known investigator of the nitriding process, no nitriding should be done at a temperature in excess of 1075 F., else the marginal layers of the nitrided zone will be brittle and tend to peel off. For this reason, most nitriding has heretofore been done below 1000 F., and while, in most instances, the nitrided zones have been found to be extremely hard, the zones are relatively thin and the time required is often as much as 100 hours.

Even when nitriding is done under the aforesaid conditions, the nitrided case is often found to be brittle. This brittleness manifests itself, for example, by the failure of the case when subjected to a too heavy impact when the supporting core is upset.

To determine if the case is brittle, several tests have been applied. One is to take a Vickers hardness reading on the nitrided surface after polishing with emery cloth. Under this condition a brittle case will spall or flake off, while a non-brittle case will show a clean cut impression. A still more drastic test consists in taking a Rockwell "no load" reading on similar surfaces. A Rockwell "no load" reading is obtained by using the Rockwell hardness tester with a diamond cone, but removing the usual 150 kilogram weight. In this condition, the load on the diamond is 60 kilograms. With this test, brittle cases will show much spalling, while the non-brittle case will not spall but may show some few radial cracks.

The toughness of the case may be determined by means of a Humphrey slow bend machine, which records the amount of work done in breaking specimens which have been nitrided. The degree of bending necessary to break the nitrided case is an indication of the relative toughness of the case.

As a result of a series of experiments, I have discovered that the brittleness of ordi-

nary nitrided cases, i. e., cases formed by nitriding at temperatures of from about 850 F. to about 1050 F. for periods up to about 100 hours, may be almost completely eliminated or cured and the toughness thereof considerably increased by heating the articles to temperatures in excess of 1100 F. but below the lower critical point of the core material, and maintaining the articles at such temperatures for periods up to about one hour.

The lower critical point of ordinary chromium-molybdenum-aluminum nitriding steels is approximately 1420 F. While heating to temperatures in excess of the lower critical point of the steel does not adversely affect the properties of the nitrided case to an appreciable degree, the physical properties of the core material may be affected or lost, and hence, it is not advisable to heat to temperatures in excess of the lower critical point. The preferred temperature is about 1200 F.

The nitrided articles are maintained at this temperature for periods up to about one hour and preferably for about one-half hour, but may be maintained at such temperature for longer periods, if desired.

In these experiments, an alloy steel containing .32% carbon, .56% manganese, .18% silicon, 1.43% chromium, .18% molybdenum and 1.30% aluminum was employed.

Specimens of this alloy steel, after being nitrided at 975° F. for about 48 hours were heated at increasing temperatures starting from 1000 F. The temperatures 1000 F. and 1100 F. had little or no effect in removing the brittleness. At 1150 and 1200 F., however, the brittleness was completely gone.

Fig. 1 of the accompanying drawings shows a Rockwell "no load" impression on a specimen of the aforementioned alloy, after being nitrided, but before heating. The marked spalling of the nitrided case may be clearly observed.

Fig. 2 shows a Rockwell "no load" impression on the same surface of the specimen as that shown in Fig. 1, but after the specimen had been heated to 1200 F. The clear cut impression shown in this figure indicates that brittleness has been substantially elim-

inated. Both figures are reproductions of microphotographs taken at 100 magnifications.

Specimens of the same alloy were also used for making the Humphrey slow bend tests to determine the toughness of the nitrided cases.

Figs. 3 and 4 are stress-strain diagrams drawn by the Humphrey machine and showing graphically the amount of work expended in breaking the specimens. The specimens for which the curve shown in Fig. 3 was obtained, were nitrided for 90 hours at 975 F. before being tested, while the specimens for which the curve shown in Fig. 4 was obtained were nitrided for 90 hours at 975 F. and then heated to 1200 F. and held at this temperature for one-half hour.

From these curves it is readily apparent that the specimens heated to 1200 F. after nitriding show a greater bend and a greater area of work done, indicating a greater toughness of case. The area under the curves is a measure of the work done in breaking the specimens.

Claims:

1. The method of decreasing the brittleness and increasing the toughness of the case of nitrided articles which consists in heating the nitrided articles to a temperature in excess of 1100 F. but below the lower critical point thereof.
2. The method of decreasing the brittleness and increasing the toughness of the case of nitrided articles which consists in heating the nitrided articles to a temperature of about 1200 F.
3. The method of providing non-brittle, tough cases on steel articles, which consists in nitriding the articles and then heating the nitrided articles to a temperature in excess of 1100 F. but below the lower critical point thereof.
4. The method of providing non-brittle, tough cases on steel articles, which consists in nitriding the articles and then heating the nitrided articles to a temperature of about 1200 F.
5. The method of providing non-brittle, tough cases on steel articles, which consists in nitriding the articles at a temperature of from about 850 F. to about 1050 F., and then heating the nitrided articles to a temperature in excess of 1100 F., but below the lower critical point of the steel.
6. The method of providing non-brittle, tough cases on steel articles, which consists in nitriding the articles at a temperature of from about 850 F. to about 1050 F., and then heating the nitrided articles to a temperature of about 1200 F.
7. The method of providing non-brittle, tough cases on steel articles, which consists in nitriding the articles at a temperature of from about 850 F. to about 1050 F. for a period varying from about 5 to about 100

hours, and then heating the nitrided articles to a temperature in excess of 1100 F. but below the lower critical point thereof.

8. The method of providing non-brittle, tough cases on steel articles, which consists in nitriding the articles at a temperature of from about 850 F. to about 1050 F. for a period varying from about 5 to about 100 hours, and then heating the nitrided articles to a temperature of about 1200 F.

In testimony whereof I affix my signature.

ROBERT SERGESON.

80

85

90

95

100

105

110

115

120

125